

Patented Mar. 9, 1926.

1,576,253

# UNITED STATES PATENT OFFICE.

LELAND L. SUMMERS, OF NEW YORK, N. Y.

## ARTIFICIAL FUEL AND THE PROCESS OF MAKING IT.

No Drawing.

Application filed September 29, 1921. Serial No. 504,148.

To all whom it may concern:

Be it known that I, LELAND L. SUMMERS, a citizen of the United States, residing at New York, in the State of New York, have 5 invented certain new and useful Improvements in Artificial Fuel and the Processes of Making It, of which the following is a specification.

My invention relates to the manufacture 10 of artificial fuel and consists in a new process by which a fuel closely resembling the characteristics of anthracite can be rapidly and cheaply made and which results in a better product than can be produced by 15 methods now in use. Such product also forms part of the invention.

The essential principle of my process is to prepare a product by utilizing carbonaceous material which has been distilled or 20 partially distilled and to cause this product to assume a dense and compact form either during the process of distillation or in a subsequent process of briquetting. The fuel so produced is subjected to an additional treatment 25 which will give it a hard protecting surface or covering by causing to be deposited on it a protecting layer of hard carbonaceous material, such covering being obtained from a solution of the bituminous 30 matter of coal in a hydrocarbon or other solvent which solution may carry carbonaceous matter of the coal in colloidal suspension. It may be deposited on the surface 35 of the fuel or forced into the fuel by pressure applied to the solution while the fuel is immersed in it. The general practice of manufacturing fuels requires the distillation of carbonaceous material to be continued to a point where a very limited amount of volatile 40 matter remains in the carbonaceous residue in order that the carbonaceous residue will withstand mechanical handling. The product thus formed is of limited use as a domestic fuel through having very little 45 volatile matter and having lost the characteristic ability of natural anthracite to ignite readily.

In my new process, the chemical and physical characteristics of anthracite may be imparted to a fuel product such as is described above. However, I prefer to make a fuel product by partially distilling bituminous coal so as to leave in the distilled product such a proportion of the volatile matter as 50 may be desired. This partially distilled coal is compressed either by briquetting or by 55 compression during the process of distillation, as is fully described in my Patents No. 943,610, December 14th, 1909, No. 1,114,065, October 20th, 1914, and No. 1,115,526, Oc- 60 tober 5th, 1915, which show various types of coking retorts for performing this function. The compressed fuel, whether partly distilled or more completely distilled, will have the chemical characteristics, the ap- 65pearance and general attributes of anthracite coal.

In carrying out my process, I do not limit myself to any particular kind or design of apparatus as many different forms can be 70 used. Nor have I considered it necessary for the purpose of this application to illustrate any apparatus at all since any apparatus alluded to herein is of a character so simple as to be readily comprehended by all 75 skilled in the art.

In the practice of my invention, I preferably form a colloidal solution of finely ground coal having its bituminous content dissolved in phenol or other hydrocarbon solvent. It is well known that coal subjected to the action of these materials is soluble so far as its bituminous matter is concerned. The fuel formed by compressing distilled carbonaceous material may be treated with 80 this solution alone or in combination with other solutions, the excess of solvent being evaporated and recovered in any manner known and practiced in the arts. I prefer- 85 ably use a solution in solvents such as phenol, cresol or creosote, and add this to the heavy residue of coal tar commonly termed pitch, the pitch being of the variety from which the volatile products have been extracted and which boils or softens only upon being high- 90 ly heated. The portion of the coal in solution to which may be added carbonaceous matter in a colloidal state is then being thoroughly mixed as in a standard auto- 95 clave. The excess solvent is then recovered 100 and the heavy solution remaining is used for the treatment of the fuel. If the fuel to be treated is slightly porous, or it is desired to increase the density of the fuel, it may be treated under pressure. For this purpose, 105 a drum or cylindrical retort such as is used in the creosoting of timber is utilized; the fuel loaded on small tram cars is run into the drum; the drum is sealed, and after exhausting the air as is done in the creosot- 110 ing of wood, the drum is filled with the hot carbonaceous mixture and steam pressure ap-

plied for a period not exceeding one hour and ordinarily about twenty minutes is sufficient. Where a coating of only slight penetration is required the treatment may be applied in an open tank. The fuel to be treated being preferably first heated is immersed in a tank of the heated carbonaceous mixture and then withdrawn and the coating allowed to harden slightly. It is then immersed again and after a few minutes immersion is withdrawn and allowed to drip while still hot. It is then allowed to cool and the coating to harden. By thus preparing the carbonaceous bath, the recovery of the solvents from the fuel after treatment is avoided as the cooling action alone will cause a hardening of the carbonaceous coating, the valuable solvents being recovered in preparing the bath or solution and the temperature of the bath being maintained at a point where it is fluid only by heat. If it is desired, similar results may be obtained by using an excess of solvents and the coating may be applied cold. The fuel after being treated will then require being subjected to a drying process preferably with the recovery of solvents in a manner well known in the arts.

In the practice of my invention I have obtained satisfactory results in using the ingredients in the following manner:

To 100 pounds of finely powdered coal, I add 50 pounds of pitch and digest this mixture with 50 pounds of phenol maintaining a temperature slightly above the boiling point of water. The mixture is then heated for two to three hours to a temperature of 225-300° F., causing the phenol to digest the soluble portions of the coal and causing the phenol to react with certain of the aldehyde bodies and other compounds to form phenolic resins. After digesting in the autoclave, I preferably add a solvent such as crude benzol or crude solvent naphtha and distill the mix-

ture for the recovery of the excess phenol. The resulting mixture is then diluted with a solvent such as crude solvent naphtha to the desired consistency and used to treat the carbonaceous material as above described. In general, a coal rich in bituminous matter is preferred and in some cases it may be desired to add a slight amount of aldehydic compounds to increase the formation of the phenolic resinous compounds in order to form a hard coating carrying the insoluble carbonaceous material of the coal in a colloidal state.

I claim:

1. The process of producing an artificial fuel which consists in subjecting raw coal to the action of a solvent for the soluble elements thereof and then covering compressed, distilled solid carbonaceous residue with the solution so obtained. 60
2. The process of producing an artificial fuel which consists in subjecting raw coal to the action of a solvent for the soluble elements thereof forming a colloidal suspension of carbon in such solvent and then covering compressed, distilled solid carbonaceous residue with such solution. 65
3. The process of producing an artificial fuel which consists in subjecting raw coal to the action of a solvent for the soluble elements thereof, mixing pitch with this solution and then covering compressed, distilled solid carbonaceous residue with the mixture so obtained. 70
4. The composition of matter for artificial fuel consisting of compressed, distilled solid carbonaceous residue covered with a solution of the soluble elements of raw coal. 80
5. The composition of matter for artificial fuel consisting of compressed, distilled solid carbonaceous residue covered with a solution of the soluble elements of raw coal mixed with carbon. 85

LELAND L. SUMMERS.